

## UNITED STATES PATENT OFFICE

2,035,518

## PROCESS FOR COLORING MATERIALS

Frithjof Zwigmeyer, Gordon Heights, Del., assignor to E. I. du Pont de Nemours & Company, Wilmington, Del., a corporation of Delaware

No Drawing. Application December 9, 1932.  
Serial No. 646,521

## 19 Claims. (Cl. 8-5)

This invention relates to processes for dyeing and printing textile fibers and more particularly refers to processes whereby fibers impregnated with ice color components are developed in such a manner that shades of exceptional and heretofore unobtainable brightness and stability may be obtained.

It is well known that insoluble azo dyestuffs may be produced on cotton and other textile material by impregnation with a suitable component followed by treatment with a diazotized aromatic amine, neither of which compounds contains a group such as carboxyl or sulfonic acid which will render the finished dyestuff water soluble. This exceedingly unsatisfactory method has recently been supplanted by a greatly improved method whereby a diazo salt is first coupled with a secondary amino compound to produce diazo-imino compounds soluble in water and/or alkali. This soluble compound mixed with a coupling component thoroughly impregnates the fibers. The secondary amino compound is then split off by treatment with suitable hydrolyzing agents, such as acetic acid, at elevated temperatures. The re-formed diazo salt immediately couples with the ice color coupling component to form insoluble dyes of improved stability and appearance.

Although this method of dyeing and printing is a tremendous advance over the prior art, nevertheless, it is subject to many disadvantages, chief among which are expensive development by treatment with steam and acid vapors; lack of uniformity of the products in many cases; noticeable dullness of the shades; low color efficiency; and corrosion of equipment.

It is an object of the present invention to avoid the objections previously enumerated and to produce colors of exceptional brightness. A further object is to produce shades having excellent stability to light and washing. A still further object is to substitute for the unsatisfactory development process which is at present practiced, a new method which is both cheap and convenient. Additional objects will appear hereinafter.

These objects are attained by the present invention wherein the impregnated material is treated with a relatively strong solution of an inert salt, preferably an alkali metal chloride such as sodium chloride, prior to or simultaneous with the hydrolysis of the impregnating substances.

The invention may be more completely under-

stood by reference to the following illustrative examples in which the quantities are stated in parts by weight:

## Example 1

A printing paste was prepared according to the following formula:

4.8 parts of the diazo-imino compound of the formula:



obtained by the action of diazotized 4-chloro-2-amino-toluene on methyl-glucamine

14.35 parts of water (160° F.)

3.0 parts of Turkey red oil

5.2 parts of the ortho-toluidide of 2:3-hydroxy-naphthoic acid

5.65 parts of sodium hydroxide solution of 30% strength

67.0 parts of thickener, made up according to the following formula:

100.0 parts wheat starch  
60 parts water  
360 parts gum tragacanth 6%

1000 parts

Cotton piece goods was printed from an engraved copper roll with the above paste, then dried. It was then treated by immersing for 20 seconds in a bath of the following composition, previously heated to 220° F. and maintained at that temperature during the development process:

1.0 part glacial acetic acid  
0.5 part formic acid, 85% strength  
28.0 parts sodium chloride  
70.5 parts water

100.0 parts

The developed printed goods was then rinsed with water, treated with a hot soap solution in the usual manner, again rinsed, then dried. The printed pattern was developed as a bright red



4.0 parts of the diazo-imino compound obtained by the action of diazotized para-toluene-azo-2:5-dimethoxy-aniline on proline, of the probable structure:



4.25 parts of the ortho-toluidide of 2:3-hydroxy-naphthoic acid  
 3.0 parts of Turkey red oil  
 21.75 parts of water (160° F.)  
 15 7.0 parts of sodium hydroxide solution of 30% strength  
 60.0 parts of thickener

100.00

20 The impregnated fiber was then immersed in the following solution, previously cooled to about 60° F.:

1.0 part glacial acetic acid  
 25 0.5 part formic acid of 85% strength  
 28.0 parts sodium chloride  
 70.5 parts water

100.0

30 The "salted and acidified" piece goods was then passed over a metal roll heated to about 220° F., suitably by passing steam through the hollow "can". This treatment results in the development of a deep blue-black dyeing, due to the 35 formation of the dyestuff of the probable structure:



50 The dyed goods was washed, soaped, rinsed and dried as in previous examples.

*Example 6*

55 Cotton piece goods was printed with a paste of the following composition:

4.6 parts of the diazo-imino compound obtained by the action of diazotized 2:5-dimethoxy-4-benzoylamino-aniline on nipecotinic-acid, of the probable formula:



70 6.3 parts of the ortho-toluidide of 2-hydroxy-anthracene-3-carboxylic acid  
 18.1 parts of water (160° F.)  
 4.0 parts of sodium hydroxide solution of 30% strength  
 70.0 parts of neutral thickener

100.0

75 The printed fiber was dried, then immersed in a cold salt-acetic-acid-formic-acid solution, as described in the previous example. The acid-

fied print was then subjected to the action of live steam, resulting in the formation of the green dyestuff of the probable structure:



15 The developed print was washed, soaped, rinsed and dried as in the previous examples.

*Example 7*

20 Cotton piece goods was printed with a paste of the following composition:

4.7 parts of the diazo-imino compound obtained by the action of diazotized 4'-ethoxy-4-amino-diphenylamine on benzyl-taurine, of the probable structure:



2.8 parts of the anilide of 2:3-hydroxy-naphthoic acid

3.0 parts of Turkey red oil

22.5 parts of water (160° F.)

7.0 parts of sodium hydroxide solution of 30% strength

60.0 parts of neutral thickener

100.0

40 The printed fiber was dried, then immersed in a boiling saturated solution of potassium chloride to which had been added 2% by weight of glacial acetic acid. When color development was complete—usually in about 30 seconds—the fiber was removed, washed, soaped, rinsed and dried. 45 The pattern was developed as a navy blue dyeing of excellent fastness properties, due to the formation of the ice color of the probable structure:



*Example 8*

60 A printing paste was prepared according to the following formula:

4.7 parts of the diazo-imino compound obtained by the action of diazotized alpha-amino-anthraquinone on monoethyl-ortho-toluidine-para-sulfonic acid, of the probable structure:



2.8 parts of the anilide of 2:3-hydroxy-naphthoic acid

5.5 parts of sodium hydroxide solution of 30% strength

5 3.0 parts of Turkey red oil  
17.0 parts of water (160° F.)  
67.0 parts of thickener

100.0

10 Cotton piece goods was printed from an engraved copper roll with the above paste, then dried. It was then immersed for one minute in a boiling saturated solution of sodium sulfate containing 1% by weight of acetic acid and 1/2% by weight of formic acid. When color development was completed, the goods was washed, soaped, rinsed and dried in the usual manner. The pattern was developed as a bright red dyeing of excellent fastness properties. The dye-stuff produced on the fiber has the probable structure:



Example 9

30 Cotton piece goods was impregnated with a paste of the following composition:

35 5.1 parts of the diazo-imino compound obtained by the action of diazotized alpha-naphthylamine on monomethyl-alpha-naphthylamine-2:4-disulfonic acid, of the probable formula:



50 3.5 parts of the anilide of 7-hydroxy-8-carboxy-alpha-naphtho-carbazole of the probable formula:



65 17.4 parts water (160° F.)  
4.0 parts sodium hydroxide solution of 30% strength  
70.0 parts thickener

100.0

70 The impregnated fiber was immersed in a saturated solution of potassium chloride, then subjected to the action of steam containing the vapors of formic acid. When color formation was completed, the goods was washed, soaped, rinsed and dried as in previous examples. A uniform

black dyeing was obtained, due to the formation of the dyestuff of the probable constitution:



Example 10

15 Cotton piece goods was printed over its entire surface from a printing roll with a paste of the following composition:

20 3.9 parts of the diazo-imino compound obtained by the action of diazotized meta-nitro-para-toluidine on the "omega-sulfonic acid" derived from para-toluidine, of the probable structure:



3.1 parts of the orthotoluidide of 2-hydroxy-carbazole-3-carboxylic acid

19.0 parts of water (160° F.)

4.0 parts of sodium hydroxide solution of 30% strength

70.0 parts of thickener

100.0 40

The printed fiber was treated with a salt acid solution, then washed, soaped and dried, as in Example 1; resulting in the dyeing of the fiber with the brown dyestuff of the probable formula:



Needless to say the components and conditions under which this process is carried out may be varied within rather wide limits without departing from the scope of the present invention. For instance, as a diazo-imino compound it may be stated in general that compounds having the following formula may be used:



in which aryl represents an aromatic residue such as a residue of the benzene, naphthalene, diphenyl, diphenylamine, anthraquinone or carbazole series free from substituents such as carboxylic or sulfonic acid groups which would render the resulting dyestuff water soluble. This com-

ponent may have substituted thereon one or more non-water solubilizing radicals, for example alkyl, alkoxy, halogen, nitro, trifluoromethyl, and acylamino groups. R represents a radical resulting from the removal of the hydrogen atom attached to the nitrogen of a secondary amine of the aliphatic, aromatic, or heterocyclic series which contains at least one water solubilizing group such as carboxylic acid, sulfonic acid, or hydroxyl.

In general, any of the coupling components common in the ice color art may be used, for instance the arylamides of 2:3-hydroxy-naphthoic acid, -hydroxy-carbazole-carboxylic acids, -hydroxy-naphtho-carbazole-carboxylic acids, and -hydroxy-anthracene-carboxylic acids; alpha- or beta-naphthol; acylacetyl-derivatives of aromatic amines; alpha-methyl-indole; and aryl-methyl-pyrazolones.

These mixtures of diazo-imino compounds and coupling components may then be imparted to the fibers in the customary manner, and in conjunction with suitable well-known assistants where necessary. Since the manner of impregnating the fibers with ice colors and the assistants commonly used therefor are well-known, enumeration of them is unnecessary and will be omitted for the sake of brevity.

As is well-known, "ice colors" may also be produced by a "one-bath" method utilizing mixtures of the arylamides of 2:3-hydroxy-naphthoic acid and nitrosamines, obtained from the bases commonly used in this art. Such a process is described in U. S. Patent 1,127,027, wherein the color is developed on the impregnated fibers by immersing in a bichromate solution. This well-known process may be modified according to the process of the present invention with excellent results. As an illustration of the means of modifying this "one-bath" process Example 1 of the aforementioned patent has been taken and the improvements of the present invention incorporated therein:

24 gms. of the anilide of 2:3-hydroxy-naphthoic acid, 40 c. c. of caustic soda lye (35° Bé.) and 50 gms. of sodium ricinoleate of 60% strength are dissolved in 150 gms. of hot water, cooled, and poured into a solution of 18 gms. of the nitrosamine-alkali metal salt of para-nitroaniline of the formula:



55 in 150 gms. of water, and 500 gms. of tragacanth thickening 1:15 are added. Cotton goods are printed with this solution, and immersed in a boiling saturated solution of sodium chloride, containing 2% by weight of acetic acid. The 60 printed fiber is rinsed, soaped, again rinsed and dried. A beautiful fast red is thereby obtained.

The application of the present invention to the "one-bath" process permits beautiful multi-colored effects to be obtained. For instance, 65 portions of the fabric may be printed with mixtures used in the "one-bath" process and different portions may be printed with mixtures containing the diazo-imino compounds described herein, the whole being simultaneously developed 70 according to the process of the present invention.

The impregnated material may be developed at somewhat elevated temperatures, temperatures somewhat above 200° F. being preferred, although in some cases, depending upon the 75 compounds being developed and other factors,

lower temperatures may be found quite satisfactory. Development according to the present invention may be carried out by several different methods according to the desires of the manufacturer and the equipment available. For instance, the dyed or printed fiber may be immersed in a strong solution of the inert salt, and the material subsequently exposed to steam and acid vapors; immersion may take place in a hot solution of the inert salt to which has been added 10 the acid required for color development; immersion may take place in a cold solution of the inert salt to which has been added the acid required for color development, and the treated material then exposed to the action of heat, for 15 example by the action of live steam or by passing the impregnated fiber over heated rolls.

The solution of inert salt described herein should contain substantially not less than 10 parts of salt per hundred parts of solution in 20 the case of salts such as sodium chloride which at this concentration would produce a reasonably strong solution, and should ordinarily be relatively saturated for optimum results. It may here be stated that the use of dilute salt 25 solutions does not permit the advantages of the present invention to be achieved, and is expressly disclaimed from the present invention. Dilute salt solutions are sometimes useful in preventing "running-out" of the printing composition prior 30 to color development. However, such solutions absolutely fail to give the excellent results obtained by the use of more concentrated solutions. Among the numerous inert inorganic salts which are known to give improved results are alkali 35 metal chlorides, alkaline earth chlorides, alkali metal sulfates, aluminum sulfate, aluminum chloride, sodium phosphates, zinc chloride and zinc sulfate. Although it may be stated that in general any inert inorganic salt may be used, 40 optimum results appear to be obtained by using a very strong solution of an alkali metal chloride. It is also possible to use mixtures of two or more salts.

Where "strong solutions" are referred to in 45 the present specification and claims it is to be understood that the lower limits of such solutions correspond in strength to a 10% solution of sodium chloride. The selection of more concentrated solutions, and preferably saturated 50 solutions, is advisable, as mentioned supra. In any event, a solution which is weaker than a 10% sodium chloride solution is not included within the meaning of the expression "strong solution".

For development of the colors various acids 55 or acid salts may be used. While the use of acetic and/or formic acid in their vapor or liquid phase is preferred, other acids may be substituted therefor among which are citric, tartaric, oxalic, and mono-chlor-acetic. In addition acid salts 60 such as sodium-dihydrogen-phosphate, potassium-hydrogen-oxalate, and sodium-hydrogen-sulfate may be substituted for the customary acetic or formic acids.

The shades produced by the herein described 65 processes are considerably brighter than those previously obtained. They are produced by a very simple treatment of the impregnated fibers with a material which is both cheap and readily available, and which does not require the use of 70 expensive equipment or exceptional skill. By the use of these processes a superior product is produced at an appreciable saving, consequently they have great commercial possibilities.

As many apparently widely different embodi- 75

ments of this invention may be made without departing from the spirit and scope thereof, it is to be understood that I do not limit myself to the specific embodiments thereof except as defined in the appended claims.

5. I claim:

1. In the process for the development of ice color printings and dyeings by subjecting to the action of an acid hydrolyzing agent fibers impregnated with mixtures of ice color coupling components and derivatives of diazotized aromatic amines which revert to the diazo salt upon treatment with the hydrolyzing agent, the step which comprises effecting hydrolysis of the impregnating material in the presence of a substantially saturated solution of an inert salt.

2. In the process for the development of ice color printings and dyeings by subjecting to the action of an acid hydrolyzing agent at elevated temperatures fibers impregnated with mixtures of ice color coupling components and derivatives of diazotized aromatic amines which revert to the diazo salt upon treatment with the hydrolyzing agent, the step which comprises effecting hydrolysis of the impregnating material in the presence of a substantially saturated solution of an inert salt selected from the group consisting of alkali metal chlorides, alkaline earth chlorides, alkali metal sulfates, aluminum sulfate, aluminum chloride, sodium phosphates, zinc chloride and zinc sulfate.

3. In the process for the development of ice color printings and dyeings by subjecting to the action of an acid hydrolyzing agent at elevated temperatures fibers impregnated with mixtures of ice color coupling components and derivatives of diazotized aromatic amines which revert to the diazo salt upon treatment with the hydrolyzing agent, the step which comprises effecting hydrolysis of the impregnating material in the presence of a strong solution of an alkali metal chloride.

4. In the process for the development of ice color printings and dyeings by subjecting to the action of an acid hydrolyzing agent at elevated temperatures fibers impregnated with mixtures of ice color coupling components and derivatives of diazotized aromatic amines which revert to the diazo salt upon treatment with the hydrolyzing agent, the step which comprises effecting hydrolysis of the impregnating material in the presence of a strong solution of sodium chloride.

5. In the process for the development of ice color printings and dyeings by subjecting to the action of an acid hydrolyzing agent at elevated temperatures fibers impregnated with mixtures of ice color coupling components and derivatives of diazotized aromatic amines which revert to the diazo salt upon treatment with the hydrolyzing agent, the step which comprises effecting hydrolysis of the impregnating material in the presence of a saturated solution of sodium chloride.

6. In the process for the development of ice color printings and dyeings by subjecting to the action of an acid hydrolyzing agent at elevated temperatures fibers impregnated with mixtures of ice color coupling components and water-soluble diazoimino compounds which revert to the diazo salt upon treatment with the hydrolyzing agent, the step which comprises effecting hydrolysis of the impregnating material in the presence of a substantially saturated solution of an inert salt.

7. In the process for the development of ice

color printings and dyeings by subjecting to the action of a dilute acid at elevated temperatures fibers impregnated with mixtures of ice color coupling components and water-soluble diazoimino compounds which revert to the diazo salt upon treatment with the hydrolyzing agent, the step which comprises effecting hydrolysis of the impregnating material in the presence of a substantially saturated solution of an inert salt selected from the group consisting of alkali metal chlorides, alkaline earth chlorides, alkali metal sulfates, aluminum sulfate, aluminum chloride, sodium phosphates, zinc chloride and zinc sulfate.

8. In the process for the development of ice color printings and dyeings by subjecting to the action of a dilute organic acid at elevated temperatures fibers impregnated with mixtures of ice color coupling components and water-soluble diazoimino compounds which revert to the diazo salt upon treatment with the hydrolyzing agent, and have the following general formula:



in which aryl represents the residue of a diazotized aromatic amine free from water-solubilizing groups, and  $\text{R}_1$  and  $\text{R}_2$  represent aromatic or aliphatic groups or together represent the residue of a heterocyclic imine at least one of which contains at least one water-solubilizing group, the step which comprises effecting hydrolysis of the impregnating material in the presence of a strong solution of an alkali metal chloride.

9. A solution for the development of ice color printings and dyeings comprising a hydrolyzing agent capable of converting derivatives of diazotized aromatic amines to their diazo salts, said solution being substantially saturated with an inert salt.

10. A solution for the development of ice color printings and dyeings comprising a hydrolyzing agent capable of converting derivatives of diazotized aromatic amines to their diazo salts, said solution being substantially saturated with an inert salt selected from the group consisting of alkali metal chlorides, alkaline earth chlorides, alkali metal sulfates, aluminum sulfate, aluminum chloride, sodium phosphates, zinc chloride and zinc sulfate.

11. A solution for the development of ice color printings and dyeings comprising a hydrolyzing agent capable of converting derivatives of diazotized aromatic amines to their diazo salts, said solution being substantially saturated with an alkali metal chloride.

12. A solution for the development of ice color printings and dyeings comprising a hydrolyzing agent capable of converting derivatives of diazotized aromatic amines to their diazo salts, said solution being substantially saturated with sodium chloride.

13. A solution for the development of ice color printings and dyeings comprising a hydrolyzing agent capable of converting derivatives of diazotized aromatic amines to their diazo salts, said solution being saturated with sodium chloride.

14. A solution for the development of ice color printings and dyeings comprising a dilute acid capable of converting the diazoimino compounds to their diazo salts, said solution being substantially saturated with an inert salt.

15. The process of claim 8 wherein the ice color coupling component is an arylamide of 2-3-hy-



CERTIFICATE OF CORRECTION.

Patent No. 2,035,518.

March 31, 1936.

FRITHJOF ZWILGMEYER.

It is hereby certified that error appears in the printed specification of the above numbered patent requiring correction as follows: Page 4, first column, line 40, in the formula, for the first "H" read N; page 6, second column, line 34, claim 8, for "presense" read presence; and that the said Letters Patent should be read with these corrections therein that the same may conform to the record of the case in the Patent Office.

Signed and sealed this 26th day of May, A. D. 1936.

Leslie Frazer

(Seal)

Acting Commissioner of Patents.